

## UNITED STATES PATENT OFFICE

1,941,231

## ALLOY OF BERYLLIUM AND ALUMINUM

Joseph Kent Smith, Detroit, Mich., assignor to  
The Beryllium Corporation, New York, N. Y.,  
a corporation of Delaware

No Drawing. Application December 22, 1931,  
Serial No. 582,658. Renewed September 1,  
1933

2 Claims. (Cl. 75—1)

This invention relates to alloys in which aluminum predominates, and to which alloys, other metals, beryllium particularly, are added not only to improve strength and mechanical characteristics, but also at once to reduce the specific gravity of the alloy and to give it greater resistance to atmospheric corrosion and similar influences.

It has long been known that the addition of beryllium to aluminum results in an alloy which is considerably lighter than is pure aluminum itself, the lessening of weight varying linearly with the beryllium content by volume. At the same time, the resistance to corrosion is considerably improved as beryllium content increases.

Because of the relatively high cost of beryllium, it is frequently desirable to keep the proportion of this element as low as possible, yet not sacrifice its valuable strengthening effects. For this reason, I have sought for combinations of metals which, added to aluminum-beryllium alloys, would intensify the effects of beryllium, and this invention relates to alloys of such type. Only those alloys higher in aluminum than in beryllium are here considered.

I have found that, by the addition of small quantities of manganese and vanadium, with or without simultaneous additions of small quantities of molybdenum, the effect of beryllium is magnified, and the resulting alloy has materially greater strength, workability, castability, bendability, as well as resistance to corrosion, than the simple binary alloy possesses. In general, I prefer compositions in which the content of aluminum and beryllium is at least ninety-five per-cent, with the aluminum running from above 55% to about 70% and the beryllium from about 25% to about 40%.

I prefer that the amounts of manganese, vanadium and molybdenum, if used, shall not be ma-

terially in excess of 5% in the aggregate, and that approximately equal amounts of each be employed—say from about  $\frac{1}{2}\%$  to about  $2\frac{1}{2}\%$ , depending upon whether molybdenum is also added.

The manganese molybdenum and vanadium, with the molybdenum if desired, as well as the beryllium for alloys low in beryllium, may be added as a master alloy, alloyed with any convenient percentage of aluminum. These metals may also be added individually directly to an aluminum-beryllium alloy previously made in any of the standard manners, or the final alloy can be formed by reduction of convenient manganese and vanadium (also molybdenum, if desired) compounds directly by the previously formed binary aluminum-beryllium alloy.

The multi-constituent alloys made in accordance with this invention are particularly well suited for castings requiring strength beyond that of ordinary aluminum, or even of its stronger alloys, like duralumin. They are also well adapted for use in sheet form, as in the case of airplane wings or fuselage parts, or wherever the combination of low specific gravity, great strength and ready bendability without breaking is essential.

I claim:

1. An alloy of approximately the following composition, aluminum from about 55% to about 70%, beryllium from about 25% to 40%, and the balance manganese molybdenum and vanadium from about  $\frac{1}{2}\%$  to  $2\frac{1}{2}\%$  each.

2. An alloy of approximately the following composition: aluminum from about 55% to about 70%, beryllium from about 25% to about 40%, the balance manganese, molybdenum and vanadium from about  $\frac{1}{2}\%$  to  $2\frac{1}{2}\%$  each but not in excess of 5.0% in the aggregate.

JOSEPH KENT SMITH. 95

60

65

70

75

80

85

90

95

100

105

110

**CERTIFICATE OF CORRECTION.**

**Patent No. 1,941,231.**

**December 26, 1933.**

**JOSEPH KENT SMITH.**

It is hereby certified that error appears in the printed specification of the above numbered patent requiring correction as follows: Line 61, strike out the word "molybdenum"; and that the said Letters Patent should be read with this correction therein that the same may conform to the record of the case in the Patent Office.

Signed and sealed this 23rd day of January, A. D. 1934.

**F. M. Hopkins**

**(Seal)**

**Acting Commissioner of Patents.**